



US006681836B1

(12) **United States Patent**  
Sakamoto et al.

(10) **Patent No.:** US 6,681,836 B1  
(45) **Date of Patent:** Jan. 27, 2004

(54) **METHOD AND APPARATUS FOR MANUFACTURING SEMI-SOLIDIFIED METAL**

5,144,998 A \* 9/1992 Hirai et al. .... 164/71.1  
5,205,981 A \* 4/1993 Fujikawa et al. .... 266/234  
5,632,801 A \* 5/1997 Lin ..... 75/708

(75) Inventors: **Kazuya Sakamoto**, Tochigi-ken (JP); **Nobumasa Hamazoe**, Kawagoe (JP); **Kenji Ohwada**, Utsunomiya (JP); **Atsushi Suzuki**, Utsunomiya (JP)

FOREIGN PATENT DOCUMENTS

(73) Assignee: **Honda Giken Kogyo Kabushiki Kaisha**, Tokyo (JP)

JP 53-131905 A 11/1978  
JP 62-130234 6/1987  
JP 01-192446 A 11/1989  
JP 2-280946 \* 11/1990  
JP 2-290931 11/1990  
JP 03-035846 A 2/1991  
JP 3-162533 7/1991  
JP 4-88135 3/1992  
JP 7-185778 7/1995  
JP 07-100589 A 8/1995  
JP 7-223047 8/1995  
WO WO 96/15867 A1 5/1996

(\*) Notice: Subject to any disclaimer, the term of this patent is extended or adjusted under 35 U.S.C. 154(b) by 0 days.

\* cited by examiner

(21) Appl. No.: **09/600,623**  
(22) PCT Filed: **Oct. 15, 1999**  
(86) PCT No.: **PCT/JP99/00163**

§ 371 (c)(1),  
(2), (4) Date: **Jul. 20, 2000**

(87) PCT Pub. No.: **WO99/36209**  
PCT Pub. Date: **Jul. 22, 1999**

(30) **Foreign Application Priority Data**

Jan. 20, 1998 (JP) ..... 10-008847  
Jan. 20, 1998 (JP) ..... 10-008849  
Jan. 20, 1998 (JP) ..... 10-008857  
Jan. 20, 1998 (JP) ..... 10-008864  
Jan. 20, 1998 (JP) ..... 10-008872

(51) **Int. Cl.<sup>7</sup>** ..... **B22D 35/06**; B22D 41/005;  
B22D 25/00  
(52) **U.S. Cl.** ..... **164/133**; 164/71.1; 164/335;  
164/900  
(58) **Field of Search** ..... 164/900, 71.1,  
164/133, 335

*Primary Examiner*—Kuang Y. Lin

(74) **Attorney, Agent, or Firm**—Birch, Stewart, Kolasch & Birch, LLP

(57) **ABSTRACT**

A predetermined amount of molten metal 12 is supplied to a heat-insulating crucible 18. After that, a chill block 46, which is cooled to a predetermined temperature of not more than a temperature of the molten metal 12, is immersed and rotated in the molten metal 12. Accordingly, the molten metal 12 is agitated while being cooled to give no directivity of cooling. It is possible to obtain semisolidified metal 20 which is formed into slurry uniformly and effectively as a whole. The semisolidified metal 20 is discharged from the heat-insulating crucible 18, and it is supplied to a forming machine 22 to apply a forming treatment thereto. Accordingly, it is possible to produce the desired slurry efficiently and economically.

(56) **References Cited**

U.S. PATENT DOCUMENTS

4,607,959 A \* 8/1986 Miyazaki et al. .... 366/343

**13 Claims, 29 Drawing Sheets**



FIG. 1  
10



FIG. 3



FIG. 4





FIG. 6 MASS PRODUCTION SYSTEM TIME TABLE



FIG. 7



FIG. 8



FIG. 9



FIG. 10





F | G.12





FIG.14



FIG.15



FIG. 16



FIG. 17



FIG. 18



FIG. 19



FIG. 20



**F I G. 21**



**F I G. 22**



FIG. 23



FIG. 24



FIG. 25



F I G. 26



FIG. 27



FIG. 28



F I G. 29



## FIG.30



FIG. 31



FIG. 32





**METHOD AND APPARATUS FOR  
MANUFACTURING SEMI-SOLIDIFIED  
METAL**

This application is the national phase under 35 U.S.C. §371 of PCT International Application No. PCT/JP99/00163 which has an International filing date of Jan. 19, 1999, which designated the United States of America.

**TECHNICAL FIELD**

The present invention relates to a method and an apparatus for producing semisolidified metal to obtain predetermined slurry from molten metal.

**BACKGROUND ART**

An operation is generally performed to produce semisolidified metal, i.e., slurry in an amount of one shot for the forming process, by using molten metal of, for example, aluminum, magnesium, or alloy thereof. It is known that a forming operation based on the use of slurry especially has such an advantage that the surface accuracy of a formed product is excellent. In order to produce such slurry, for example, the thixocasting process and the rheocasting process are widely adopted.

However, in the case of the thixocasting process described above, it is necessary to use an exclusive billet and a reheating apparatus. For this reason, the following problems are pointed out. That is, the material cost and the equipment cost are considerably expensive, and the entire production operation is complicated.

On the other hand, in the rheocasting process, the mass production is performed based on the continuous batch system. In this process, the cooling is performed by discharging the molten metal while allowing the molten metal to make contact with a cooling section cooled with water. Therefore, the temperature of slurry differs between the start and the end of the cooling. A problem arises in that the temperature of the slurry is not managed accurately.

A method is also known, in which slurry is produced in accordance with cooling, heating, and agitation in a forming machine. However, the following inconveniences arise. That is, the cycle time is prolonged, and especially the shot weight is increased.

When the produced slurry is supplied into the forming machine, a container for accommodating the slurry is usually inverted in the vertical direction. However, it is difficult to discharge the entire amount of slurry in the container, for example, due to the temperature of the slurry in the container, the shape of the container, and the weight of the slurry. As a result, the following problems are pointed out. That is, remaining matters of the slurry appear in the container, and the supply weight of the slurry is dispersed. Further, the slurry, which is newly produced in the container, is badly affected thereby.

When different parts are formed, the shot weight differs depending thereon. Therefore, the following problems are pointed out. That is, it is impossible to correctly manage the temperature of the slurry. When the shot weight is increased, it takes a long time to perform the operation for producing the slurry. It is difficult to efficiently perform the forming operation for a variety of different parts to give high qualities.

An object of the present invention is to provide a method and an apparatus for producing semisolidified metal, which make it possible to produce desired slurry efficiently and economically.

Another object of the present invention is to provide an apparatus for producing semisolidified metal, which makes it possible to economically produce desired slurry and easily discharge the slurry in a reliable manner.

Still another object of the present Invention is to provide an apparatus for producing semisolidified metal, which makes it possible to economically produce various slurries having different weight so that they have high qualities, wherein the system is simplified.

**DISCLOSURE OF THE INVENTION**

According to the present invention, a predetermined amount of molten metal is supplied to a heat-insulating crucible. After that, the molten metal in the crucible is cooled by the aid of a cooling member which is cooled to be at a predetermined temperature of not more than a temperature of the molten metal. Simultaneously, the molten metal is agitated. Accordingly, in the heat-insulating crucible, the molten metal is reliably formed into slurry generally uniformly as a whole without involving any directivity of cooling. Thus, the reheating is unnecessary, and it is possible to efficiently obtain desired semisolidified metal.

According to the present invention, a predetermined amount of molten metal is supplied to a heat-insulating crucible, and then the molten metal in the crucible is cooled by the aid of a cooling member which is cooled to be at a predetermined temperature of not more than a temperature of the molten metal. Further, the cooling member is moved in the horizontal direction and/or in the vertical direction while rotating the cooling member. Thus, the molten metal is agitated. For example, the cooling member is moved in a reciprocating manner in the horizontal direction and/or in the vertical direction. Alternatively, the cooling member is moved spirally in the horizontal direction.

Accordingly, especially when heat-insulating crucibles having various shapes are used, the cooling member is moved along with the shape of the heat-insulating crucible. Thus, the directivity of cooling is excluded to be as less as possible, and the molten metal can be effectively agitated.

Accordingly, the molten metal is formed into slurry uniformly and reliably as a whole. It is possible to obtain desired semisolidified metal efficiently with a high quality.

In the present invention, the semisolidified metal is produced after a predetermined amount of molten metal is supplied to a heat-insulating crucible, by cooling and agitating the molten metal in the heat-insulating crucible by the aid of a plurality of cooling members. Accordingly, even when the shot weight is increased, then the directivity of cooling is avoided to be as less as possible, and it is possible to quickly and smoothly obtain the desired semisolidified metal formed into slurry uniformly and reliably as a whole.

Further, the cooling members are integrally held by a driving mechanism by the aid of a fixing means in a state in which an arbitrary number of the cooling members are stacked with each other. Therefore, it is enough to change the number of stacked cooling members depending on the change of the shot weight. Thus, it is possible to produce the desired semisolidified metal efficiently to have a high quality. The fixing means includes a shaft member for being integrally inserted into the plurality of stacked cooling members, and a fixture for being screwed on an end of the shaft member. Thus, it is possible to effectively simplify the structure.

In the present invention, the molten metal is supplied into a heat-insulating crucible, and then a cooling member is immersed in the molten metal. The molten metal is agitated

in a state in which a cooling medium having a predetermined temperature is supplied to the inside of the cooling member. Accordingly, the directivity of cooling is avoided to be as less as possible, and it is possible to convert the molten metal into slurry quickly and reliably. Further, when the temperature of the cooling medium is managed, it is unnecessary to reheat the semisolidified metal. Thus, it is possible to efficiently obtain the desired semisolidified metal.

In the present invention, a predetermined amount of molten metal is supplied to divided type heat-insulating crucibles. After that, the molten metal in the heat-insulating crucibles is cooled and agitated by the aid of a cooling member to produce semisolidified metal. Subsequently, the heat-insulating crucibles are subjected to opening/closing operation by the aid of an opening/closing mechanism. Accordingly, the semisolidified metal in the heat-insulating crucibles falls in accordance with its self-weight, and it is discharged from the heat-insulating crucibles.

Accordingly, the directivity of cooling is avoided to be as less as possible, and it is possible to obtain the desired semisolidified metal formed into slurry uniformly and reliably as a whole. Further, it is possible to discharge the semisolidified metal from the heat-insulating crucibles smoothly and reliably.

#### BRIEF DESCRIPTION OF THE DRAWINGS

FIG. 1 shows an illustrative schematic perspective view depicting a production apparatus for carrying out a method for producing semisolidified metal according to a first embodiment of the present invention.

FIG. 2 shows an illustrative plan view depicting the production apparatus.

FIG. 3 illustrates the operation of a molten metal-ladling robot which constructs the production apparatus.

FIG. 4 illustrates an agitator which constructs the production apparatus.

FIGS. 5A to 5E illustrate a chill block-treating unit for treating a chill block which constructs the agitator.

FIG. 6 shows a time table for a mass production system based on the use of the production apparatus.

FIG. 7 illustrates the temperature change of each of portions in a crucible during the operation of the production apparatus.

FIG. 8 shows an illustrative perspective view depicting the operation of the production apparatus.

FIG. 9 shows an illustrative perspective view depicting the operation of the production apparatus.

FIG. 10 shows an illustrative schematic perspective view depicting a production apparatus for carrying out a method for producing semisolidified metal according to a second embodiment of the present invention.

FIGS. 11A to 11F show steps illustrating the operation of the production apparatus.

FIG. 12 shows an illustrative schematic perspective view depicting a production apparatus for carrying out a method for producing semisolidified metal according to a third embodiment of the present invention.

FIGS. 13A to 13G show steps illustrating the operation of the production apparatus.

FIG. 14 illustrates a chill block having a cylindrical configuration.

FIG. 15 illustrates a chill block having a bottom-equipped cylindrical configuration.

FIG. 16 shows an illustrative schematic perspective view depicting a production apparatus for carrying out a method

for producing semisolidified metal according to a fourth embodiment of the present invention.

FIG. 17 illustrates an agitator which constructs the production apparatus.

FIG. 18 shows an illustrative schematic perspective view depicting the agitator.

FIG. 19 shows an illustrative schematic perspective view depicting an agitator which constructs a production apparatus for carrying out a method for producing semisolidified metal according to a fifth embodiment of the present invention.

FIG. 20 shows an illustrative schematic perspective view depicting an agitator which constructs a production apparatus for carrying out a method for producing semisolidified metal according to a sixth embodiment of the present invention.

FIG. 21 illustrates a chill block designed to have an external shape of an elliptical configuration.

FIG. 22 illustrates a chill block designed to have an external shape of a composite elliptical configuration.

FIG. 23 illustrates a chill block designed to have an external shape of a chamfered rectangular configuration.

FIG. 24 illustrates a chill block designed to have an external shape of a hexagonal configuration.

FIG. 25 illustrates a chill block designed to have an external shape of a chamfered hexagonal configuration.

FIG. 26 shows an illustrative schematic perspective view depicting an apparatus for producing semisolidified metal according to a seventh embodiment of the present invention.

FIG. 27 illustrates an agitator which constructs the production apparatus.

FIG. 28 illustrates, in cross section, chill blocks which construct the agitator.

FIG. 29 shows an illustrative schematic perspective view depicting an apparatus for producing semisolidified metal according to an eighth embodiment of the present invention.

FIG. 30 illustrates a chill block which constructs an apparatus for producing semisolidified metal according to a ninth embodiment of the present invention.

FIG. 31 shows an illustrative schematic view, with partial cross section, depicting an apparatus for producing semisolidified metal according to a tenth embodiment of the present invention.

FIG. 32 illustrates a magnified view depicting a cooling member which constructs the production apparatus.

FIG. 33A illustrates a step of supplying molten metal to a crucible.

FIG. 33B illustrates a step of raising the crucible to immerse the cooling member in the molten metal.

FIG. 33C illustrates a step of supplying first liquid metal to the cooling member to cool and agitate the molten metal.

FIG. 33D illustrates a step of supplying second liquid metal to the cooling member after the semisolidified metal is produced.

#### BEST MODE FOR CARRYING OUT THE INVENTION

FIG. 1 shows an illustrative schematic perspective view depicting a production apparatus 10 for carrying out a method for producing semisolidified metal according to the first embodiment of the present invention, and FIG. 2 shows an illustrative plan view depicting the production apparatus 10.

The production apparatus **10** comprises a molten metal-holding furnace **14** for holding molten metal **12** which is composed of melted metal such as aluminum, alloy thereof, magnesium, and alloy thereof; a molten metal-ladling robot **16** for ladling a predetermined amount (amount for one shot) of the molten metal **12** from the molten metal-holding furnace **14**; a supply robot **26** for pouring the molten metal **12** ladled by the molten metal-ladling robot **16** into a predetermined heat-insulating crucible **18**, and supplying semisolidified metal **20** formed into a desired slurry state in the crucible **18** to a slurry-introducing port **24** which communicates with an unillustrated cavity of a forming machine **22**; and first to fourth agitators **28a** to **28d** each of which is arranged for the crucible **18** for cooling and agitating the molten metal **12** in the crucible **18**.

As shown in FIGS. 1 and 3, the molten metal-ladling robot **16** includes an arm **32** which is provided swingably on a support pillar **30**. A ladle **34** is installed tiltably to the forward end of the arm **32**. The supply robot **26** is movable back and forth along a rail **36** which extends in a direction (direction of the arrow **A**) of arrangement of the first to fourth agitator **28a** to **28d**. The supply robot **26** is an articulated type robot, and it has, at its forward end, a gripping section **38** capable of holding the heat-insulating crucible **18**.

The first agitator **28a** includes a crucible holder **40** on which the crucible **18** is detachably arranged. As shown in FIG. 4, the crucible holder **40** is provided with a recess **42** for accommodating the crucible **18**. A heater **44** is embedded at the inside of the crucible holder **40** so that the heater **44** circumscribes the crucible **18** arranged in the recess **42**.

A chill block (cooling member) **46**, which also has an agitating function, is detachably arranged with a driving mechanism **48** at a position over the crucible holder **40**. The chill block **46** is made of, for example, a material such as copper and stainless steel which is not melted at the molten temperature of aluminum molten metal to be used as the molten metal **12**. The external shape of the chill block **46** is designed to have a columnar configuration, with a draft sloped downwardly.

The chill block **46** is detachable with respect to a driving mechanism **48** by the aid of a coupler **49** made of ceramics. The driving mechanism **48** is moved upwardly and downwardly over the crucible holder **40**, and it drives and rotates the chill block **46**.

The second to fourth agitators **28b** to **28d** are constructed in the same manner as the first agitator **28a** described above. The same constitutive components are designated by the same reference numerals, detailed explanation of which will be omitted.

Each of the chill blocks **46** is detachable with respect to each of the driving mechanisms **48** provided for the first to fourth agitators **28a** to **28d**. The chill block **46** is detached from the driving mechanism **48** every time when the molten metal **12** is agitated and cooled (for every one shot), and it is fed to a chill block-treating unit **50**.

As shown in FIGS. 5A to 5E, the chill block-treating unit **50** comprises a cooling tank **52** for cooling the chill block **46** disengaged from the driving mechanism **48** with a cooling medium such as cooling oil; an air blow means **54** for effecting air blow against the chill block **46** after the cooling to remove solidified matters of aluminum from the surface; a coating tank **56** for immersing the chill block **46** after the air blow in a coating liquid composed of a ceramic material; and a drying means **60** for drying the chill block **46** after the coating with a heater **58**.

The operation of the production apparatus **10** constructed as described above will be explained below. FIG. 6 shows a time table for the mass production system based on the use of the production apparatus **10**.

At first, the molten metal-ladling robot-**16** is operated in a state in which the molten metal **12** is heated and maintained at about 650° C. in the molten metal-holding furnace **14**. As shown in FIG. 3, the molten metal-ladling robot **16** is operated as follows. That is, the ladle **34** is inserted into the molten metal-holding furnace **14** in accordance with the action of the arm **32**. The ladle **34** is inclined or tilted, so that the molten metal **12** in an amount of one shot is ladled by the ladle **34**. The ladle **34**, which has ladled the molten metal **12**, is moved to a pouring position (see the position depicted by two-dot chain lines in FIG. 3). On the other hand, the supply robot **26**, which holds the empty crucible **18**, is arranged at the pouring position by the aid of the gripping section **38** (see FIG. 1).

In this situation, the ladle **34** is tilted, and the molten metal **12** in the amount of one shot is poured into the crucible **18** held by the supply robot **26**. Subsequently, the supply robot **26** inserts the crucible **18** at a predetermined position of each of the first to fourth agitators **28a** to **28d**, for example, into the recess **42** of the crucible holder **40** which constitutes the first agitator **28a**. The heater is operated in the crucible holder **40** to maintain a predetermined temperature beforehand. The molten metal **12** in the crucible **18** arranged in the recess **42** is prevented from being cooled all at once by the surroundings.

In the first agitator **28a**, the chill block **46** is previously heated and maintained at about 100° C. in order to remove any moisture and stabilize the cooling condition. The chill block **46** is immersed in the molten metal **12** in the crucible **18** while being rotated in a predetermined direction at a relatively low speed by the aid of the driving mechanism **48**. After that, the rotation speed of the chill block **46** is increased in the molten metal **12** in accordance with the action of the driving mechanism **48**. Thus, the molten metal **12** is quickly agitated while being cooled.

After the chill block **46** agitates the molten metal **12** for a preset period of time or until a slurry-supply signal is inputted, the chill block **46** is raised and withdrawn from the crucible **18** while being rotated. Accordingly, the semisolidified metal **20**, which is maintained to have a constant temperature as a whole, is obtained in the heat-insulating crucible **18**.

Changes occur as shown in FIG. 7 in the steps for producing the semisolidified metal **20** described above, concerning the atmosphere in the crucible **18**, the temperature of the crucible **18**, the center temperature of the molten metal **12**, the end temperature of the molten metal **12**, and the temperature of the chill block **46**.

On the other hand, the supply robot **26** is moved, for example, corresponding to the fourth agitator **28d** which possesses the semisolidified metal **20** cooled and agitated to give a desired slurry state, of the first to fourth agitators **28a** to **28d**. In the fourth agitator **28d**, the driving mechanism **48** waits at an upward position, and the chill block **46** is removed. The supply robot **26** grips the crucible **18** which is arranged on the crucible holder **40** of the fourth agitator **28d**, and it takes the crucible **18** out of the fourth agitator **28d** (see FIG. 8).

The supply robot **26** is further operated such that the crucible **18**, which is gripped by the gripping section **38**, is arranged with respect to the slurry-introducing port **24** of the forming machine **22**, and then the crucible **18** is inverted.

Accordingly, the semisolidified metal **20** in the crucible **18** is allowed to fall so that it falls to be supplied to the slurry-introducing port **24** (see FIG. 9). In the forming machine **22**, the forming process is performed with the semisolidified metal **20** to obtain a predetermined formed product.

The supply robot **26** moves the empty crucible **18** to the air blow position to apply the air blow treatment thereto. Accordingly, any aluminum, which remains in the heat-insulating crucible **18**, is removed. Subsequently, the inside of the crucible **18** is subjected to coating with a ceramic material or the like, and then the crucible **18** is arranged at the pouring position.

In the first agitator **28a**, the chill block **46**, which is retracted upwardly after performing the cooling and the agitation for the molten metal **12**, is disengaged from the driving mechanism **48**, and it is transported to the chill block-treating unit **50** by the aid of a robot or the like (see FIG. 5A). In the chill block-treating unit **50**, as shown in FIG. 5B, the chill block **46** is firstly immersed in the cooling tank **52** to perform the cooling treatment. After that, the air blow means **54** is used to remove aluminum solidified matters adhered to the surface of the chill block **46** (see FIG. 5C). Further, as shown in FIG. 5D, the chill block **46** is immersed in a coating liquid in the coating tank **56** to coat the surface thereof with a ceramic material, because of the following reason. That is, the surface of the chill block **46** is prevented from any reaction with the molten metal **12**, and it is easy to remove aluminum solidified matters adhered to the surface of the chill block **46**.

The chill block **46** after the coating treatment is subjected to the drying treatment in accordance with the action of the heater **58** which constitutes the drying means **60**. The chill block **46** is heated to a predetermined temperature (see FIG. 5E). After the drying, the chill block **46** is installed to the driving mechanism **48**, and it is used again to perform the cooling and agitating operations for the new molten metal **12**.

In the first embodiment of the present invention, the molten metal **12** in the crucible **18** is cooled by using the chill block **46** which is maintained at the temperature lower than the temperature of the molten metal **12**. The chill block **46** is rotated to effect the agitation. Accordingly, no directivity occurs during the cooling of the molten metal **12**. It is possible to obtain the semisolidified metal **20** formed into the slurry uniformly and reliably as a whole. It is possible to supply the semisolidified metal **20** to the slurry-introducing port **24** of the forming machine **22** without heating the semisolidified metal **20** again.

As a result, it is possible to always obtain the stable semisolidified metal **20** for every one shot. Further, it is unnecessary to provide any equipment such as the reheating apparatus. Accordingly, the effect can be obtained such that it is possible to produce the semisolidified metal **20** economically and efficiently. Further, the external shape of the chill block **46** is designed to have the columnar configuration. It is possible to effectively prevent the chill block **46** from being deteriorated by the molten metal **12** formed into the slurry. The chill block **46** has the draft which is sloped downwardly. Accordingly, it is possible to smoothly withdraw the chill block **46** from the semisolidified metal **20**.

In the first embodiment, the air blow means **54** is used to remove the aluminum solidified matters adhered to the surface of the chill block **46**. However, in place of the air blow means **54**, it is possible to use, for example, a vibration-generating means and a sandblast means.

In the first embodiment, the molten metal-ladling robot **16** for ladling the molten metal in the amount of one shot is provided between the molten metal-holding furnace **14** and the supply robot **26**. However, it is not necessarily indispensable to use the molten metal-ladling robot **16** provided that the apparatus is constructed such that the molten metal **12** in the amount of one shot is directly fed from the molten metal-holding furnace **14** to the crucible **18** held by the supply robot **26**.

FIG. 10 shows an illustrative schematic perspective view depicting a production apparatus **70** for carrying out a method for producing semisolidified metal according to the second embodiment of the present invention.

The production apparatus **70** comprises divided type crucibles **80a**, **80b**; divided type crucible holders **82a**, **82b** for accommodating the crucibles **80a**, **80b**; a molten metal-feeding means **86** for feeding molten metal **84** into the crucibles **80a**, **80b**; an agitator **88** for cooling and agitating the molten metal **84** in the crucibles **80a**, **80b**; and a supply robot **92** for integrally holding the crucibles **80a**, **80b** to take them out of the crucible holders **82a**, **82b**, and feeding semisolidified metal **90** to the forming machine **22**.

The crucibles **80a**, **80b** are constructed by dividing a bottom-equipped cylinder into two in the diametral direction. A pair of hook-shaped projections **94a**, **94b** and a pair of grooves **96a**, **96b** are arranged linearly in the axial direction on the outer circumferences of the crucibles **80a**, **80b** respectively (see FIG. 11A). A heat-resistance packing **97** is interposed between joining surfaces of the crucibles **80a**, **80b**.

As shown in FIG. 11A, the crucible holders **82a**, **82b** are constructed by dividing a bottom-equipped cylinder into two in the diametral direction. The crucible holders **82a**, **82b** are swingably supported at supporting points **98a**, **98b** of their respective lower end angular portions with respect to an installation plane **99**. Rods **102a**, **102b**, which extend from cylinders **100a**, **100b**, are connected to side portions of the crucible holders **82a**, **82b**, while the cylinders **100a**, **100b** are tiltable with respect to the installation plane **99**.

When the crucible holders **82a**, **82b** are closed, a recess **104** is integrally formed therein. Heaters **106a**, **106b** are embedded to circumscribe the recess **104**.

As shown in FIG. 10, the molten metal-feeding means **86** is provided with a ladle **108** for ladling the molten metal **84** in an amount of one shot from the molten metal-holding furnace **14**. The ladle **108** is constructed tiltably and movably between the ladling position for the molten metal **84** and the pouring position for the crucibles **80a**, **80b**.

The agitator **88** is provided with a chill block (cooling member) **110** which is made of, for example, stainless steel. The external shape of the chill block **110** is designed to have a columnar configuration. The chill block **110** is rotatable and movable upwardly and downwardly by the aid of an unillustrated driving mechanism. The chill block **110** is inserted rotatably into a lid member **112**. The lid member **112** is movable upwardly and downwardly in an integrated manner together with the chill block **110**. It is desirable that the lid member **112** is made of a material having no gas permeability. The surface, which makes contact with the molten metal **84**, is designed to be a planar surface or to have a conical or pyramidal configuration protruding toward the molten metal **84** at its central portion.

The supply robot **92** is provided with a wrist section **114**. An opening/closing mechanism **115** is installed to the wrist section **114**. The opening/closing mechanism **115** has cylinders **116a**, **116b** which serve as forward/backward moving

means. Ends of arm members **120a**, **120b** disposed vertically downwardly are secured to rods **118a**, **118b** which extend in mutually opposite directions from the cylinders **116a**, **116b**. The arm members **120a**, **120b** are provided with a pair of outer projections **122a**, **122b** which are inserted into and engaged with the respective projections **94a**, **94b** of the crucibles **80a**, **80b**, and a pair of inner projections **124a**, **124b** which are fitted to the grooves **96a**, **96b** of the crucibles **80a**, **80b**.

A lid member **126**, which is positioned under the opening/closing mechanism **115** and which is made of a heat-insulating material, is secured to the supply robot **92**. The lid member **126** makes tight contact with the upper surfaces of the crucibles **80a**, **80b** to ensure the heat-insulating performance of the crucibles **80a**, **80b** when the crucibles **80a**, **80b** are held by the arm members **120a**, **120b**. The lid member **126** also functions to avoid any leakage of the semisolidified metal **90**.

In the second embodiment constructed as described above, the crucibles **80a**, **80b** are firstly inserted between the crucible holders **82a**, **82b** in a state in which the crucible holders **82a**, **82b** are mutually open to stand on the supporting points **98a**, **98b** as shown in FIG. 11A. Subsequently, the cylinders **100a**, **100b** are operated to displace the rods **102a**, **102b** frontwardly respectively. Accordingly, the crucible holders **82a**, **82b** make swinging movement in directions to make approach to one another. Therefore, the crucibles **80a**, **80b** are accommodated in the recess **104** which is formed integrally between the crucible holders **82a**, **82b**. In this arrangement, the size of the recess **104** is designed to be slightly smaller than the external shape of the crucibles **80a**, **80b**. The crucibles **80a**, **80b** are held in a liquid-tight manner with each other with the heat-resistance packings **97** intervening therebetween in a state in which the crucible holders **82a**, **82b** are mutually closed.

Subsequently, as shown in FIG. 11B, the ladle **108**, which constitutes the molten metal-feeding means **86**, ladles the molten metal **84** in the amount of one shot, and the molten metal **84** is fed into the crucibles **80a**, **80b**. The crucibles **80a**, **80b** are heated and held at a predetermined temperature (for example, 280° C.) by the aid of the heaters **106a**, **106b** embedded in the crucible holders **82a**, **82b**. The molten metal **84**, which is aluminum molten metal maintained at 650° C. to 700° C., is fed into the crucibles **80a**, **80b**.

On the other hand, in the agitator **88**, the chill block **110** is heated to 100° C. in order to remove, for example, moisture. As shown in FIG. 11C, the chill block **110** is moved downwardly from a position over the crucibles **80a**, **80b** while being rotated. Accordingly, the chill block **110** cools the molten metal **84** in the crucibles **80a**, **80b**, and it agitates the molten metal **84**. More preferably, the chill block **110** is immersed in the molten metal **84** in the crucibles **80a**, **80b** while being rotated in a predetermined direction at a relatively low speed. After that, the rotation speed of the chill block **110** is increased in the molten metal **84**. Accordingly, the chill block **110** quickly agitates the molten metal **84** while cooling the molten metal **84**.

During this process, the lid member **112** is moved downwardly integrally with the chill block **110**. The lid member **112** is arranged on the open upper end side of the crucibles **80a**, **80b**. Accordingly, the surface of the molten metal **84** is not oxidized during the cooling and the agitation effected by the chill block **110**. Further, it is possible to reliably avoid any contamination of air into the molten metal **84**.

The cooling and the agitation are performed for a predetermined period of time to obtain the semisolidified metal **90**.

in a desired slurry state. After that, the chill block **110** is taken out of the crucibles **80a**, **80b** while being rotated. On the other hand, the supply robot **92** is arranged over the crucibles **80a**, **80b**. The supply robot **92** is operated such that the arm members **120a**, **120b** are moved downwardly by the aid of the wrist section **114** (see FIG. 11D). The respective outer projections **122a**, **122b** are fitted to the projections **94a**, **94b** of the crucibles **80a**, **80b**. The respective inner projections **124a**, **124b** are fitted to the grooves **96a**, **96b** of the crucibles **80a**, **80b**.

Subsequently, as shown in FIG. 11E, the crucible holders **82a**, **82b** make swinging movement in directions to make separation from each other in accordance with the action of the cylinders **100a**, **100b**. The crucibles **80a**, **80b**, which have been held by the recess **104**, are taken out in a state of being held by the arm members **120a**, **120b**. The wrist section **114** is arranged at a position over the slurry-introducing port **24** of the forming machine **22**. After that, the cylinder **116a**, **116b**, which construct the opening/closing mechanism **115**, are operated to displace the rods **118a**, **118b** in directions to make separation from each other.

Therefore, the arm members **120a**, **120b** are displaced in directions to make separation from each other. The crucibles **80a**, **80b**, which are held by the arm members **120a**, **120b**, are released from each other. The semisolidified metal **90** is produced integrally in the crucibles **80a**, **80b**. When the crucibles **80a**, **80b** are open, then the semisolidified metal **90** falls, and it is supplied to the slurry-introducing port **24** (see FIG. 11F).

As described above, in the second embodiment, the molten metal **84** in the amount of one shot, which is fed into the crucibles **80a**, **80b**, are agitated in accordance with the rotating action of the chill block **110** while being cooled by the chill block **110**. Accordingly, it is possible to obtain the semisolidified metal **90** in a satisfactory slurry state, which has no directivity of cooling and which is uniform as a whole. Further, the open ends of the crucibles **80a**, **80b** are closed by the lid member **112** during the cooling and the agitation effected by the chill block **110**. Therefore, it is possible to effectively avoid any oxidation of the surface of the molten metal **84** and any contamination of air into the molten metal **84**. Accordingly, such an effect is obtained that the semisolidified metal **90** having a high quality can be efficiently obtained.

The apparatus further includes the divided type crucibles **80a**, **80b**. The arm members **120a**, **120b**, which constitute the robot **92**, are engaged with the crucibles **80a**, **80b** respectively so that the crucibles **80a**, **80b** may be opened and closed. Accordingly, the semisolidified metal **90** is reliably allowed to fall, and it can be easily supplied to the slurry-introducing port **24** merely by moving the crucibles **80a**, **80b** in the directions to make separation from each other at the position over the slurry-introducing port **24**.

Therefore, in the second embodiment, the entire amount of the semisolidified metal **90** can be reliably discharged from the crucibles **80a**, **80b** with the simple arrangement without being affected, for example, by the temperature of the semisolidified metal **90** in the crucibles **80a**, **80b**, the shape of the crucibles **80a**, **80b**, and the weight of the semisolidified metal **90**. Accordingly, the supply weight of the semisolidified metal **90** is not dispersed, which would be otherwise caused by the occurrence of any remaining matter of the semisolidified metal **90** in the crucibles **80a**, **80b**. Further, such an effect is obtained that it is possible to effectively prevent the semisolidified metal **90** to be newly produced in the crucibles **80a**, **80b** from being badly affected.

FIG. 12 shows an illustrative schematic perspective view depicting a production apparatus 130 for carrying out a method for producing semisolidified metal according to the third embodiment of the present invention.

The production apparatus 130 comprises divided type crucibles 140a, 140b; divided type crucible holders 142a, 142b; a robot 144 for transporting the crucibles 140a, 140b; a molten metal-feeding means 148 for feeding molten metal 146 in an amount of one shot into the crucibles 140a, 140b; and an agitator 150 for cooling and agitating the molten metal 146 in the crucibles 140a, 140b.

A pair of projections 152a, 152b are formed to expand on outer circumferential portions of the crucibles 140a, 140b. The crucible holder 142a is connected to a rod 158 which extends from a cylinder 156, and it is movable back and forth in directions of the arrow by the aid of a pulley 160. The crucible holder 142b is fixed to an installation plane 161. When the crucible holders 142a, 142b are mutually closed, a recess 162 is integrally formed therein. Heaters 164a, 164b are embedded in the crucible holders 142a, 142b respectively (see FIG. 13A).

An opening/closing mechanism 166 is installed to the robot 144. Upper ends of arm members 172a, 172b are connected to rods 170a, 170b which extend from cylinders 168a, 168b for constructing the opening/closing mechanism 166. Fastening means 174a, 174b, which are used to make engagement with the projections 152a, 152b provided on the side surfaces of the crucibles 140a, 140b, are provided on lower end sides of the arm members 172a, 172b.

The molten metal-feeding means 148 is provided with a ladle 176. The agitator 150 is provided with a chill block 178 having a relatively small diameter. The chill block 178 is rotatable by the aid of a driving mechanism 180. The driving mechanism 180 is installed to a movable base 182, and it is movable in the direction of the arrow (in the horizontal direction).

In the third embodiment constructed as described above, the operation is firstly performed as shown in FIG. 13A. That is, in a state in which the crucible holder 142a is separated from the crucible holder 142b, the crucibles 140a, 140b are gripped by the robot 144, and they are inserted into the crucible holders 142a, 142b. Subsequently, the crucible holder 142a is moved toward the crucible holder 142b to be mutually closed in accordance with the driving action of the cylinder 156. The crucibles 140a, 140b are accommodated and held in the recess 162 which is integrally formed therebetween (see FIG. 13B).

Further, as shown in FIG. 13C, the molten metal 146 in the amount of one shot is fed into the crucibles 140a, 140b by the aid of the ladle 176 which constitutes the molten metal-feeding means 148. After that, as shown in FIG. 13D, the agitator 150 is operated. In the agitator 150, the chill block 178, which is cooled at a predetermined temperature, is rotated by the aid of the driving mechanism 180 while being immersed in the molten metal 146. The movable base 182 is moved back and forth in the horizontal direction. Accordingly, the molten metal 146 in the crucibles 140a, 140b is cooled and agitated to obtain the semisolidified metal 184 having a desired slurry state.

Subsequently, as shown in FIG. 13E, the arm members 172a, 172b, which construct the robot 144, enter the inside of the crucible holders 142a, 142b to grip the crucibles 140a, 140b. After that, the crucible holder 142a is operated to be open in accordance with the action of the cylinder 156, while the robot 144 is moved upwardly (see FIG. 13F). The robot 144 arranges the crucibles 140a, 140b corresponding to the

predetermined slurry-introducing port 24. When the arm members 172a, 172b make swinging movement in directions to make separation from each other in accordance with the action of the cylinders 168a, 168b, then the crucibles 140a, 140b mutually make swinging movement in opening directions, and thus the semisolidified metal 184 falls to be supplied to the slurry-introducing port 24 (see FIG. 13G).

Therefore, in the third embodiment, the same effect as that of the second embodiment is obtained by using the divided type crucibles 140a, 140b.

In the first to third embodiments, the chill blocks 46, 110, 178 are designed to have the columnar configuration. However, it is enough that at least the external shape has the columnar configuration. For example, a chill block 186 shown in FIG. 14 includes a cylindrical member 188, and an attachment plate 189 to which an end of the cylindrical member 188 is secured. A chill block 190 shown in FIG. 15 includes a bottom-equipped cylindrical member 192, and a shaft member 194 which is secured to an inner bottom portion 192a of the cylindrical member 192.

FIG. 16 shows an illustrative schematic perspective view depicting a production apparatus 200 for carrying out a method for producing semisolidified metal according to the fourth embodiment of the present invention. The same 25 constitutive components as those of the production apparatus 70 according to the second embodiment shown in FIG. 10 are designated by the same reference numerals, detailed explanation of which will be omitted.

The production apparatus 200 is provided with an agitator 202. As shown in FIGS. 16 and 17, a chill block (cooling member) 204, which constructs the agitator 202, is detachably arranged with respect to a rotary section 206 with a 30 coupler 208 made of ceramics intervening therebetween, at a position over crucible holders 82a, 82b. The chill block 204 is composed of, for example, a material such as copper and stainless steel which is not melted at a melting temperature of aluminum molten metal to be used as the molten metal 84. The external shape of the chill block 204 is 35 designed to have a quadratic prism-shaped configuration, with a draft formed downwardly.

The rotary section 206 rotates and drives the chill block 204. The rotary section 206 is constructed to be movable upwardly and downwardly in an integrated manner together with the chill block 204 by the aid of a moving section 210, and it is moved along a spiral configuration in the horizontal 40 direction (see FIG. 18). That is, the moving section 210 has two functions of an elevator means and a spiral movable means. A driving mechanism is constructed by the rotary section 206 and the moving section 210.

As shown in FIG. 18, in the production apparatus 200 according to the fourth embodiment constructed as described above, the molten metal 84 in the crucibles 80a, 80b is cooled by the chill block 204 which is maintained at a temperature lower than the temperature of the molten metal 84. The molten metal 84 is agitated by moving the chill block 204 in the spiral configuration in the horizontal direction along the shape of the crucibles 80a, 80b while rotating the chill block 204. Accordingly, no directivity occurs during the cooling of the molten metal 84 in the 50 crucibles 80a, 80b. It is possible to quickly obtain the desired semisolidified metal 90 formed into the slurry uniformly and reliably as a whole. Therefore, it is unnecessary to reheat the semisolidified metal 90. The semisolidified metal 90 can be directly supplied to the slurry-introducing port 24 of the forming machine 22.

Accordingly, the following effects are obtained. That is, it is possible to always obtain the stable semisolidified metal

90 for every one shot. Further, it is unnecessary to provide the equipment such as the reheating unit, and it is possible to produce the semisolidified metal 90 economically and efficiently. The external shape of the chill block 204 is designed to have the quadratic prism-shaped configuration. Therefore, it is possible to reliably agitate the molten metal 84. The chill block 204 has the draft formed downwardly. Thus, the chill block 204 can be smoothly withdrawn from the semisolidified metal 90.

FIG. 19 shows an illustrative schematic perspective view depicting an agitator 290 which constructs a production apparatus for carrying out a method for producing semisolidified metal according to the fifth embodiment of the present invention.

The agitator 290 is provided with a pair of chill blocks (cooling members) 296a, 296b for cooling and agitating molten metal 294 in divided type crucibles 292a, 292b. The chill blocks 296a, 296b are arranged detachably with respect to rotary sections 298a, 298a with couplers 300a, 300b made of ceramics intervening therebetween. The chill blocks 296a, 296b are made of, for example, copper or stainless steel, in the same manner as the chill block 204. The chill blocks 296a, 296b are designed to have a quadratic prism-shaped external shape, and they have a draft formed downwardly.

The rotary sections 298a, 298b rotate and drive the chill blocks 296a, 296b. On the other hand, the rotary sections 298a, 298b are movable upwardly and downwardly in an integrated manner together with the chill blocks 296a, 296b by the aid of a moving section 302, and they make reciprocating movement in the horizontal direction along the longitudinal direction (direction of the arrow A) of the crucibles 292a, 292b. That is, the moving section 302 has two functions of an elevator means and a horizontally moving means.

The crucibles 292a, 292b are designed to have a rectangular configuration in a state of making tight contact with each other. A heat-resistant packing 304 is interposed between their joining surfaces. The crucibles 292a, 292b are arranged on unillustrated divided type crucible holders. An integrated type crucible may be adopted in place of the divided type crucibles 292a, 292b.

In the fifth embodiment constructed as described above, the molten metal 294 in an amount of one shot is firstly fed into the inside of the crucibles 292a, 292b which are allowed to make tight contact with each other. After that, the chill blocks 296a, 296b are arranged at positions over the crucibles 292a, 292b by the aid of the moving section 302. Subsequently, the chill blocks 296a, 296b are moved downwardly while being rotated in accordance with the action of the rotary sections 298a, 298b.

The chill blocks 296a, 296b are moved in a reciprocating manner in the horizontal direction in accordance with the action of the moving section 302, after the chill blocks 296a, 296b are immersed in the molten metal 294 in the crucibles 292a, 292b, or simultaneously with the rotary driving. Accordingly, the chill blocks 296a, 296b cool the molten metal 294 in the crucibles 292a, 292b, and they agitate the molten metal 294 along the shape of the crucibles 292a, 292b.

As described above, in the fifth embodiment, the chill blocks 296a, 296b make the reciprocating movement along the longitudinal direction (direction of the arrow A) of the crucibles 292a, 292b while being rotated. Accordingly, the molten metal 294 can be agitated reliably and effectively over the entire interior of the crucibles 292a, 292b.

Therefore, the same effects as those obtained in the fourth embodiment are obtained, for example, such that it is possible to obtain the desired semisolidified metal 90 in the satisfactory slurry state which is uniform as a whole and which has no directivity of cooling, in the crucibles 292a, 292b.

FIG. 20 shows an illustrative schematic perspective view depicting an agitator 320 which constructs a production apparatus for carrying out a method for producing semisolidified metal according to the sixth embodiment of the present invention.

The agitator 320 is provided with a chill block (cooling member) 326 for cooling and agitating molten metal 324 in divided type crucibles 322a, 322b. The chill block 326 is arranged detachably with respect to a, rotary section 328 with a coupler 330 made of ceramics intervening therebetween. The chill block 326 is made of, for example, copper or stainless steel, in the same manner as the chill block 204 described above. The chill block 326 is designed to have a quadratic prism-shaped external shape, and it has a draft formed downwardly.

A rotary section 328 rotates and drives the chill block 326. On the other hand, the rotary section 328 is movable upwardly and downwardly in an integrated manner together with the chill block 326 by the aid of a moving section 332. That is, the moving section 332 has a function to serve as a vertically moving means for making reciprocating movement of the chill block 326 in the longitudinal direction (direction of the arrow B) of the crucibles 322a, 322b.

The crucibles 322a, 322b are designed to have a cylindrical configuration in a state of making tight contact with each other. A heat-resistant packing 334 is interposed between their joining surfaces. The crucibles 322a, 322b are arranged on unillustrated divided type crucible holders. An integrated type crucible may be adopted in place of the divided type crucibles 322a, 322b.

In the sixth embodiment constructed as described above, the molten metal 324 in an amount of one shot is firstly fed into the inside of the crucibles 322a, 322b which are allowed to make tight contact with each other. After that, the chill block 326 is arranged at a position over the crucibles 322a, 322b by the aid of the moving mechanism 332.

Subsequently, the chill block 326 is moved downwardly by the aid of the moving section 332 while being rotated in accordance with the action of the rotary section 328. The chill block 326 is immersed in the molten metal 324 in the crucibles 322a, 322b, and then it makes reciprocating movement in the vertical direction in accordance with the action of the moving section 332. Accordingly, the chill block 326 cools the molten metal 324 in the crucibles 322a, 322b, and it agitates the molten metal 324 along the shape of the crucibles 322a, 322b.

As described above, in the sixth embodiment, the chill block 326 makes the reciprocating movement in the longitudinal direction (direction of the arrow B) of the crucibles 322a, 322b while being rotated. Accordingly, the molten metal 324 can be agitated reliably and effectively over the entire interior of the crucibles 322a, 322b. Therefore, the same effects as those obtained in the fourth and fifth embodiments are obtained, for example, such that it is possible to obtain the desired semisolidified metal 90 in the satisfactory slurry state which is uniform as a whole and which has no directivity of cooling.

In the fourth to sixth embodiments, each of the chill blocks 204, 296a, 296b, 326 is designed to have the rectangular configuration. However, there is no limitation

thereto. For example, it is also allowable to use a chill block 340 designed to have an external shape of an elliptical configuration (see FIG. 21), a chill block 342 designed to have an external shape of a composite elliptical configuration (see FIG. 22), a chill block 344 designed to have an external shape of a chamfered rectangular configuration (see FIG. 23), a chill block 346 designed to have an external shape of a hexagonal configuration (see FIG. 24), and a chill block 346 designed to have an external shape of chamfered hexagonal configuration (see FIG. 25).

FIG. 26 shows an illustrative schematic perspective view depicting an apparatus 400 for producing semisolidified metal according to the seventh embodiment of the present invention. The same constitutive components as those of the production apparatus 200 according to the fourth embodiment shown in FIG. 16 are designated by the same reference numerals, detailed explanation of which will be omitted.

The production apparatus 400 is provided with an agitator 402. A plurality of chill blocks (cooling members) 406a to 406d, which construct the agitator 402, are detachably connected to a rotary section 206 with a coupler 208 made of ceramics intervening therebetween, at a position over crucible holders 82a, 82b. The chill blocks 406a to 406d are composed of, for example, a material such as copper and stainless steel which is not melted at a melting temperature of aluminum molten metal to be used as the molten metal 84. As shown in FIGS. 26 to 28, the external shape of the entire chill blocks 406a to 406d is designed to have a quadratic prism-shaped configuration, with a draft formed downwardly.

As shown in FIG. 28, through-holes 408a to 408d are formed at respective central portions of the chill blocks 406a to 406d. An arbitrary number of the chill blocks 406a to 406d can be held in an integrated manner with respect to the rotary section 206 by the aid of a fixing means 412. The fixing means 412 includes a screw shaft (shaft member) 414 for being integrally inserted into the through-holes 408a to 408d of the stacked chill blocks 406a to 406d, a nut member (fixture) 416 for being screwed on the lower end of the screw shaft 414, and a support plate 415 for supporting the chill blocks 406a to 406d. The upper end of the screw shaft 414 can be detachably connected to the coupler 208.

In the case of the production apparatus 400 constructed as described above, when the weight of the molten metal 84 in the amount of one shot is changed depending on the change of the part to be formed, the number of chill blocks 406a to 406d installed to the rotary section 206 is increased or decreased. Specifically, when the weight of the molten metal 84 in the amount of one shot is decreased, the chill blocks 406a to 406d are decreased, for example, to the chill blocks 406a to 406c. On the other hand, when the weight of the molten metal 84 in the amount of one shot is increased, a predetermined number of chill blocks (not shown) may be stacked on the chill blocks 406a to 406d.

As described above, in the seventh embodiment, the molten metal 84 in the crucibles 80a, 80b is cooled with the predetermined number of chill blocks 406a to 406d, and the chill blocks 406a to 406d are rotated in an integrated manner by the aid of the rotary section 206 to agitate the molten metal 84. Accordingly, the following effects are obtained. That is, no directivity occurs during the cooling of the molten metal 84 in the crucibles 80a, 80b. It is possible to extremely quickly and efficiently obtain the desired semisolidified metal 22 formed into the slurry uniformly and reliably as a whole.

Further, when the weight of the molten metal 84 in the amount of one shot is changed, it is enough that the number

of chill blocks 406a to 406d is increased or decreased depending on the weight of the molten metal 84. It is possible to efficiently and highly accurately produce the semisolidified metal 90 for forming a variety of different parts. Accordingly, the following advantages are obtained. That is, it is unnecessary to prepare any exclusive cooling means corresponding to the change of the weight of the molten metal 84. It is possible to effectively reduce the equipment cost.

FIG. 29 shows an illustrative schematic perspective view depicting an apparatus 490 for producing semisolidified metal according to the eighth embodiment of the present invention. The same constitutive components as those of the production apparatus 400 according to the seventh embodiment are designated by the same reference numerals, detailed explanation of which will be omitted.

The production apparatus 490 includes a plurality of chill blocks (cooling members) 492a to 492d which also possess the agitating function. The chill blocks 492a to 492d are detachably arranged with respect to the driving mechanism 494 with a coupler 496 made of ceramics intervening therebetween. The chill blocks 492a to 492d are made of, for example, copper or stainless steel, and their upper ends are integrated into one unit with a connecting section 498. The connecting section 498 is detachable with respect to the coupler 496. The external shape of each of the chill blocks 492a to 492d is designed to have a columnar configuration, and each of the chill blocks 492a to 492d has a draft formed downwardly.

In the eighth embodiment constructed as described above, the molten metal 84 in an amount of one shot is fed into the crucibles 80a, 80b. After that, the chill blocks 492a to 492d are moved downwardly while being rotated by the aid of the driving mechanism 494, and they are immersed in the molten metal 84 in the crucibles 80a, 80b. Accordingly, the molten metal 84 in the crucibles 80a, 80b is cooled and agitated to obtain the semisolidified metal 90 having a desired slurry state.

Accordingly, in the eighth embodiment, the four chill blocks 492a to 492d are operated in an integrated manner to agitate the molten metal 84 while cooling the molten metal 84 in the crucibles 80a, 80b. Therefore, even when the weight of the molten metal 84 is especially large, an effect is obtained such that the desired semisolidified metal 90 can be obtained efficiently and quickly.

FIG. 30 illustrates a chill block 500 which constructs an apparatus for producing semisolidified metal according to the ninth embodiment of the present invention.

The chill block 500 is provided with a plurality of rib sections 504a to 504i which are integrally formed on the outer circumference of a columnar section 502 while being separated from each other by predetermined spacing distances in the axial direction. Therefore, in the ninth embodiment, when the chill block 500 is rotated in the molten metal 84, the molten metal 84 is cooled and agitated quickly and smoothly by the aid of the plurality of rib sections 504a to 504i. Thus, it is possible to obtain the same effects as those obtained in the seventh and eighth embodiments.

FIG. 31 shows an illustrative schematic view, with partial cross section, depicting an apparatus 510 for producing semisolidified metal according to the tenth embodiment of the present invention.

The production apparatus 510 comprises a heat-insulating crucible 514 for holding molten metal 512 composed of melted metal in a predetermined amount (amount of one

shot); a coil-shaped cooling member 516 for cooling the molten metal 512 in the crucible 514 to a predetermined temperature; a cooling mechanism 520 for supplying, to the inside of the cooling member 516, first liquid metal 518 as a cooling medium maintained at a temperature which is not more than the temperature of the molten metal 512; and an electromagnetic agitation mechanism (driving mechanism) 522 for agitating the molten metal 512 by the aid of the cooling member 516.

The crucible 514 is made of, for example, silicon nitride. The crucible 514 is arranged on an elevator base 524. A heating heater 526 is installed to the outer circumference of the crucible 514. The elevator base 524 is movable upwardly and downwardly by the aid of an unillustrated driving means, and it is designed to be rotatable, if necessary. A coil section 528, which constructs the electromagnetic agitation mechanism 522, is arranged to surround the crucible 514 in the vicinity of the elevator base 524.

The cooling mechanism 520 includes a first supply means 530 for supplying first liquid metal 518 into the cooling member 516 in order to cool the molten metal 512 to a predetermined temperature, and a second supply means 534 for supplying, into the cooling member 516, second liquid metal 532 which is a heating medium having a temperature higher than a liquefying temperature of solidified matters in order to remove the solidified matters adhered to the surface of the cooling member 516. The molten metal 512 is melted metal composed of, for example, aluminum, alloy thereof, magnesium, or alloy thereof. The first and second liquid metals 518, 532 are stannum or stannum alloy.

The first supply means 530 includes a first storage tank 536 for storing the first liquid metal 518; a first heating furnace (first heating section) 538 for keeping the temperature of the first liquid metal 518 in the first storage tank 536; a heat exchanger 540 for cooling the first liquid metal 518 by performing heat exchange with respect to the first liquid metal 518; and a first circulating passage 542 for circulating the first liquid metal 518 through the inside of the cooling member 516.

The heat exchanger 540 is provided with a heat exchange coil 544 for supplying cooling water thereinto. The heat exchange coil 544 is immersed in the first liquid metal 518 in the first storage tank 536. The first heating furnace 538 is arranged to circumscribe the first storage tank 536. The first circulating passage 542 is composed of a pipe made of SUS. An inlet end 542a thereof is connected to a lower end side of the first storage tank 536. An outlet end 542b thereof is immersed at a predetermined height position in the first liquid metal 518 at an upward portion of the first storage tank 536. As shown in FIG. 32, the first circulating passage 542 constitutes a part of the cooling member 516. A first electromagnetic pump 546 is arranged on the side of the end 542a (see FIG. 31).

The second supply means 534 includes a second storage tank 548 for storing the second liquid metal 532; a second heating furnace (second heating section) 550 for heating the second liquid metal 532 in the second storage tank 548; and a second circulating passage 552 for circulating the cooling member 532 through the inside of the cooling member 516.

The second heating furnace 550 is arranged to circumscribe the second storage tank 548. The second circulating passage 552 has its inlet end 552a which is joined to the lower side of the second storage tank 548, and its outlet end 552b which is immersed at a predetermined position in the second liquid metal 532 at an upper portion of the second storage tank 548. A second electromagnetic pump 554 is

provided for the second circulating passage 552 in the vicinity of the side of the end 552a. The second circulating passage 552 is joined with the first circulating passage 542 at its intermediate portion to constitute a part of the cooling member 516 (see FIG. 32).

A first thermocouple (first detecting means) 558 for measuring the temperature of the molten metal is installed at the joined portion of the first and second circulating passages 542, 552 by the aid of a support member 556. The first thermocouple 558 detects the temperature of the molten metal 512 in the crucible 514. A second thermocouple (second detecting means) 560 for detecting the temperature of the first liquid metal 518 is arranged for the first storage tank 536 which constructs the first supply means 530. On the other hand, a third thermocouple (third detecting means) 562 for detecting the temperature of the second liquid metal 532 is arranged for the second storage tank 548 which constructs the second supply means 534.

Explanation will be made below for the operation of the production apparatus 510 according to the tenth embodiment constructed as described above.

At first, the operation is performed as shown in FIG. 33A. That is, for example, the molten metal 512 of aluminum alloy (AC2B), which is used as a material for the molten metal, is held at a temperature of 650°C. in an unillustrated molten metal-holding furnace. A feeder 564 ladles the molten metal 512 in an amount of one shot, for example, in an amount of 20 kg to be fed to the crucible 514. The heater 526 is installed to the crucible 514. The temperature of the molten metal 512 in the crucible 514 is maintained to be constant by the aid of the heater 526.

Subsequently, as shown in FIG. 33B, the elevator base 524, on which the crucible 514 is placed, is moved upwardly. The cooling member 516 is immersed in the molten metal 512 in the crucible 514. The cooling member 516 is a pipe made of SUS having an inner diameter of 20 mm, which is constructed to have a coil-shaped configuration with an entire length of 700 mm.

On the other hand, in the cooling mechanism 520, as shown in FIG. 31, the first liquid metal 518 is maintained at 250°C., and it is stored in an amount of 100 liters in the first storage tank 536 which constitutes the first supply means 530. The second liquid metal 532 is maintained at 600°C., and it is stored in an amount of 40 liters in the second storage tank 548 which constitutes the second supply means 534. The temperatures of the first and second liquid metals 518, 532 are detected by the second and third thermocouples 560, 562 respectively. The heat exchanger 540 and the first heating furnace 538 are operated on the basis of the result of the detection performed by the second thermocouple 560. Thus, the temperature of the first liquid metal 518 is maintained to be constant. On the other hand, the second heating furnace 550 is operated on the basis of the result of the detection performed by the third thermocouple 562. Thus, the temperature of the second liquid metal 532 is maintained to be constant.

The first electromagnetic pump 546 is operated so that the first liquid metal 518 in the first storage tank 536 is introduced into the inside of the cooling member 516 via the first circulating passage 542 at a flow rate of 20 liters/minute. After that, the first liquid metal 518 is returned from the end 542b to the inside of the first storage tank 536 (see FIG. 33C). Accordingly, the molten metal 512 in the crucible 514 is cooled by the aid of the cooling member 516 in which the first liquid metal 518 having the relatively low temperature is circulated through the inside. During this process, the coil

section 528, which constitutes the electromagnetic agitation mechanism 522, is operated to agitate the molten metal 512 in the crucible 514.

The temperature of the molten metal 512 in the crucible 514 is detected by the first thermocouple 558. The cooling and the agitation are performed for the molten metal 512 until the detected temperature arrives at the preset semisolidification temperature. Therefore, the semisolidified metal 566, which has no directivity of cooling and which is formed into the slurry uniformly and successfully as a whole, is produced in the crucible 514 (see FIGS. 31 and 33C).

Subsequently, the operation of the first electromagnetic pump 546 is stopped, and the second electromagnetic pump 554 is operated. Accordingly, as shown in FIG. 33D, the liquid metal 532 in the second storage tank 548 is supplied to the inside of the cooling member 516 via the second circulating passage 552 at a flow rate of 20 liters/minute. The second liquid metal 532 is held at a temperature higher than the liquefaction temperature of the aluminum alloy used for the molten metal 512. Even when aluminum solidified matters adhere to the surface of the cooling member 516, the aluminum solidified matters can be dissolved again to reliably remove them. After that, the operation of the second electromagnetic pump 554 is stopped, and the elevator base 524 is moved downwardly to separate the crucible 514 from the cooling member 516.

Accordingly, the desired semisolidified metal 566 is obtained in the crucible 514. During this process, the first and second liquid metals 518, 532 are supplied to the cooling member 516 at the flow rate of 20 liters/minute by the aid of the first and second electromagnetic pumps 546, 554. Therefore, the molten metal 512 in the crucible 514 is cooled from 650°C. to the slurry temperature of 570°C. for about 1 minute. On the other hand, it is possible to effectively prevent the surface of the cooling member 516 from adhesion of aluminum solidified matters.

In the tenth embodiment, the first liquid metal 518, which is maintained at the predetermined cooling temperature, is supplied in the circulating manner to the inside of the cooling member 516 to cool the molten metal 512 in the state in which the cooling member 516 is immersed in the molten metal 512 in the crucible 514. Further, the electromagnetic agitation mechanism 522 is operated to agitate the molten metal 512. Accordingly, no directivity occurs during the cooling of the molten metal 512. It is possible to obtain the semisolidified metal 566 formed into the slurry uniformly and reliably as a whole.

The first and second thermocouples 558, 560 are used to detect the temperatures of the molten metal 512 and the first liquid metal 518 so that the temperature of the first liquid metal 518 is managed. Accordingly, it is unnecessary to reheat the semisolidified metal 566. Such an effect is obtained that the semisolidified metal 566 having a high quality can be efficiently obtained. Especially, it is advantageous that the temperature of the semisolidified metal 566 is managed easily and correctly, and the cooling speed for the molten metal 512 is improved so that the semisolidified metal 566 may be quickly produced all at once.

The tenth embodiment is provided with the second supply means 534 for supplying, to the inside of the cooling member 516, the second liquid metal 532 having the temperature higher than the liquefaction temperature of the molten metal material (for example, aluminum alloy) after the semisolidified metal 566 is produced. That is, it is feared that the aluminum solidified matters formed by the solidification of the molten metal 512 adhere to the surface of the

cooling member 516 after performing the cooling and the agitation for the molten metal 512, resulting in formation of any solidified layer. If the solidified layer has a thick wall thickness, then it is feared that the aluminum solidified matters are oxidized to cause contamination into the molten metal 512 in the crucible 514 upon the next time shot, or the aluminum solidified matters cause the change of the cooling condition of the molten metal 512 and the dispersion of the amount of the molten metal.

In the tenth embodiment, the second liquid metal 532 having the relatively high temperature is supplied to the second circulating passage 552. Therefore, the aluminum solidified matters, which adhere to the surface of the cooling member 516, are dissolved again, and they are reliably removed from the surface. Accordingly, it is possible to efficiently obtain the semisolidified metal 566 having the high quality, and it is possible to stabilize the cooling condition.

In the tenth embodiment, the cooling member 516 is designed to have the coil-shaped configuration in which the first and second circulating passages 542, 552 are joined to one another in the integrated manner. However, the cooling member 516 may be designed to have various configurations such as a plate-shaped configuration, for example, corresponding to the volume and the shape of the crucible 514. That is, the cooling member 516 may be designed to have an optimum configuration so that the surface area is increased.

The electromagnetic agitation mechanism 522 is used to agitate the molten metal 512. However, in place thereof, it is possible to adopt a mechanical agitation structure. For example, the molten metal 512 may be agitated by rotating the crucible 514 itself, or by moving the crucible 514 in the horizontal direction together with the rotation of the crucible 514. Further, the following arrangement is also available. That is, the cooling member 516 itself may be rotated, or it may be designed to be movable in the horizontal direction.

#### INDUSTRIAL APPLICABILITY

As described above, in the present invention, the molten metal, which is supplied to the heat-insulating crucible, is agitated while being cooled by the aid of the cooling member. Therefore, the molten metal is formed into the slurry in the crucible uniformly and reliably as a whole. It is possible to easily and efficiently obtain the desired semisolidified metal having no directivity of cooling. Further, it is unnecessary to reheat the semisolidified metal. It is possible to reliably avoid the expensive equipment cost.

In the present invention, the molten metal in the crucible is cooled by the aid of the cooling member, and the molten metal is agitated by moving the cooling member along the shape of the crucible. Accordingly, the molten metal is formed into the slurry in the heat-insulating crucible uniformly and reliably as a whole. It is possible to easily and efficiently obtain the desired semisolidified metal having no directivity of cooling.

In the present invention, the molten metal in the crucible is cooled and agitated by the aid of the plurality of cooling members. Therefore, the directivity of cooling is excluded to be as less as possible, and it is possible to quickly and efficiently produce the desired semisolidified metal formed into the slurry uniformly and reliably as a whole.

In the present invention, the cooling member is immersed in the molten metal in the heat-insulating crucible. The molten metal is agitated in the state in which the cooling medium is supplied to the inside of the cooling member. Accordingly, no directivity occurs during the cooling of the

## 21

molten metal, and it is possible to form the slurry of the molten metal quickly and reliably. Further, the desired semisolidified metal can be obtained efficiently and highly accurately by managing the temperature of the cooling medium.

In the present invention, the molten metal, which is contained in the divided type heat-insulating crucibles, is cooled and agitated by the aid of the cooling member to produce the semisolidified metal. After that, the heat-insulating crucibles are subjected to the opening/closing operation by the aid of the opening/closing mechanism. Accordingly, the semisolidified metal in the heat-insulating crucibles falls from the heat-insulating crucibles due to its own weight, and it is discharged therefrom. Accordingly, the directivity of cooling is excluded to be as less as possible, and it is possible to obtain the desired semisolidified metal formed into the slurry uniformly and reliably as a whole. Further, it is possible to discharge the semisolidified metal from the heat-insulating crucibles smoothly and reliably by using the simple structure.

What is claimed is:

1. A method for producing semisolidified metal, comprising the steps of:

supplying a predetermined amount of molten metal to a heat-insulating non-cooled crucible;  
 cooling said molten metal in said heat-insulating crucible by the aid of a cooling member used as an agitator, said cooling member being cooled to a predetermined temperature which is not more than a temperature of said molten metal, and agitating said molten metal;  
 agitating said molten metal by using said cooling member;  
 completing said agitation step after agitating said molten metal to give a predetermined slurry state;  
 withdrawing said cooling member to a position outside of said heat-insulating crucible;  
 subjecting said cooling member to a temperature control process in a cooling member treating unit;  
 removing solidified matters adhered to a surface of said cooling member after withdrawing said cooling member from said heat-insulating crucible;  
 coating said cooling member with a ceramic material after removing said solidified matters; and  
 applying a drying treatment to said cooling member after coating said cooling member with said ceramic material prior to moving the cooling member to a position inside the heat-insulating crucible.

2. A method for producing semisolidified metal, comprising the steps of:

supplying a predetermined amount of molten metal to a heat-insulating crucible;  
 cooling said molten metal in said heat-insulating crucible by the aid of a cooling member cooled to a predetermined temperature which is not more than a temperature of said molten metal, said cooling member being displaceable from a position outside of said heat-insulating crucible to a position inside said heat-insulating crucible;  
 agitating said molten metal by moving said cooling member in a horizontal direction and/or in a vertical direction while rotating said cooling member;  
 completing said agitation step after agitating said molten metal to give a predetermined slurry state;  
 withdrawing said cooling member to said position outside of said heat-insulating crucible; and

## 22

tilting said crucible so that said molten metal in said predetermined slurry state falls into a forming unit, wherein the step of supplying the predetermined amount of molten metal to a heat-insulating crucible is performed concurrently with the step of agitating said molten metal in at least two other heat-insulating crucible.

3. The method for producing said semisolidified metal according to claim 1, wherein an external shape of said cooling member is set to have a columnar configuration with a draft formed downwardly.

4. The method for producing said semisolidified metal according to claim 1, wherein an external shape of said cooling member is set to have a prism configuration with a draft formed downwardly.

5. The method for producing said semisolidified metal according to claim 1 or 2, wherein said cooling member is inserted into said heat-insulating crucible, and an open end of said heat-insulating crucible is closed by a lid member.

6. The method for producing said semisolidified metal according to claim 1 or 2, wherein a plurality of cooling members are provided.

7. An apparatus for producing semisolidified metal, comprising:

a heat-insulating crucible for holding predetermined amount of molten metal;  
 a cooling member for agitating and cooling said molten metal in said heat-insulating crucible to a predetermined temperature;  
 means for displacing said cooling member from a position outside of said heat-insulating crucible to a position inside said heat-insulating crucible;  
 a driving mechanism for agitating said molten metal by rotating said cooling member;  
 first temperature control means for controlling temperature of said cooling member after displacing said cooling member to said position outside said heat-insulating crucible;  
 air blow means for removing semi solidified metal from the cooling member;  
 coating means for applying a coat of ceramic material to a surface of the cooling member; and  
 drying mean for subjecting the cooling member to a drying treatment prior to displacing the cooling member to said position inside the heat-insulating crucible.

8. The apparatus for producing said semisolidified metal according to claim 7, wherein an external shape of said cooling member is set to have a columnar configuration with a draft formed downwardly.

9. An apparatus for producing semisolidified metal, comprising:

means for successively supplying a predetermined amount of molten metal into each of a plurality of heat-insulating crucibles;  
 a cooling member for each of said heat-insulating crucibles for agitating and cooling said molten metal to a predetermined temperature;  
 means for displacing said cooling members from a positions outside of said heat-insulating crucibles to positions inside said heat-insulating crucibles;  
 a driving mechanism for agitating said molten metal by moving said cooling members in a horizontal direction and/or in a vertical direction while rotating said cooling member;  
 wherein the means for supplying molten metal to one of the heat-insulating crucible operates concurrently with

the agitating and cooling operation of the cooling members of at least two others of the heat-insulating crucibles.

10. The apparatus for producing said semisolidified metal according to claim 9, wherein said driving mechanism includes a horizontal moving means for making reciprocating movement of said cooling members in said horizontal direction.

11. The apparatus for producing said semisolidified metal according to claim 9, wherein said driving mechanism includes a spiral moving means for making spiral movement of said cooling members in said horizontal direction.

12. The apparatus for producing said semisolidified metal according to claim 9, wherein said driving mechanism includes a vertical moving means for making reciprocating movement of said cooling members in said vertical direction.

13. The apparatus for producing said semisolidified metal according to claim 9, wherein an external shape of each of the said cooling members is set to have a prism configuration with a draft formed downwardly.

\* \* \* \* \*

UNITED STATES PATENT AND TRADEMARK OFFICE  
**CERTIFICATE OF CORRECTION**

PATENT NO. : 6,681,836 B1  
DATED : January 27, 2004  
INVENTOR(S) : Sakamoto et al.

Page 1 of 1

It is certified that error appears in the above-identified patent and that said Letters Patent is hereby corrected as shown below:

Title page,  
Item [22], PCT Filed, change “**October 15, 1999**” to -- **January 19, 1999** --.

Signed and Sealed this

Fourteenth Day of September, 2004

A handwritten signature in black ink, appearing to read "Jon W. Dudas", is placed within a rectangular box with a dotted grid background.

JON W. DUDAS  
*Director of the United States Patent and Trademark Office*